

T. HANCOCK.

MANUFACTURE OF METAL REFLECTORS, MIRRORS, AND OTHER METAL ARTICLES HAVING A  
REFLECTING SURFACE OR SURFACES.

APPLICATION FILED MAY 3, 1918.

1,336,224.

Patented Apr. 6, 1920.



Fig. 1.



Fig. 2.



Fig. 3.



Fig. 4.

INVENTOR:

By *Thomas Hancock*  
*McMullan Mfg.*

# UNITED STATES PATENT OFFICE.

THOMAS HANCOCK, OF BOW, ENGLAND, ASSIGNOR TO THE REFLECTO-METAL COMPANY, LIMITED, OF LONDON, ENGLAND.

## MANUFACTURE OF METAL REFLECTORS, MIRRORS, AND OTHER METAL ARTICLES HAVING A REFLECTING SURFACE OR SURFACES.

1,336,224.

Specification of Letters Patent.

Patented Apr. 6, 1920.

Application filed May 3, 1918. Serial No. 232,252.

*To all whom it may concern:*

Be it known that I, THOMAS HANCOCK, a subject of the King of Great Britain and Ireland, residing at 108 The Grove, Bow, 5 in the county of Essex, England, have invented new and useful Improvements in the Manufacture of Metal Reflectors, Mirrors, and other Metal Articles Having a Reflecting Surface or Surfaces, of which the following is a specification.

The invention relates to the manufacture of metal reflectors or mirrors, that is to say of articles having a reflecting surface, and consists of a method by which such articles 15 can be cheaply and expeditiously manufactured.

The method of manufacture consists in momentarily dipping into a bath of a metal or alloy, formers which are provided with a smooth and highly polished surface that is the reverse of the reflecting surface of the reflectors or mirrors to be produced, whereby a film of metal adheres to the surface of the former and solidifies thereon.

In carrying out the invention a former is made with a smooth and highly polished surface, which is made of a shape the reverse of the reflecting surface of the reflector or mirror to be made. For instance, in the case of a parabolic reflector the main part of the former, that is to say the part which determines the shape of the article to be manufactured, would consist of a head made of a shape the reverse of the inner surface of the parabolic reflector, while the remainder of the former would consist of a connected stem. The necessary former having been made, a bath of the metal or alloy to be used is prepared, and is maintained, 40 during the process of manufacture, at a constant temperature, which is slightly above the melting point of the metal or alloy. After the removal of the scum from the surface of the bath of metal, so that a perfectly clean and bright metal surface is 45 presented to the former, the head of the former is dipped into the bath of molten metal to a depth such that the part of the former which determines the shape of the article to be manufactured is immersed in the bath. The former is then immediately withdrawn, and will be found to be covered with a coating of the metal. The former with its adherent coating is allowed to cool,

and this quickly takes place. On separation from the former the coating or shell will be found to have a surface highly polished where previously in contact with the highly polished surface of the former. When the former has become cooled its 60 polished surface is carefully wiped to render it clean and bright for use again in the manner described.

The metal shells formed as above described, after their rough edges have been removed, and, if necessary, cut to any particular shape, may be secured to backings of stout metal or be otherwise used according to circumstances.

In practice a number of formers may be 70 employed so as to enable a relatively great number of articles to be manufactured at a time.

The former is made of a material, adapted to take a high polish and to withstand the 75 heat of the bath of molten metal. Thus the former cools the metal in contact with its immersed surface. Materials from which the formers may be made are for example annealed glass, porcelain and china, particularly the first named.

The metals or alloys which may be utilized in the manufacture of the reflectors or mirrors, apart from the fact that they must be capable of having a reflecting surface imparted to them, must be such that they will be cooled at the surface of contact with the former and must be such that the coating produced will not develop cracks or fissures as it cools. Metals and alloys which can be 85 employed are for example those of low melting point such as tin, an alloy of tin and lead containing a small percentage of copper, antimony or other metal which will exert a hardening effect on the tin, or tin 90 and lead and prevent deterioration of the reflecting surface under normal atmospheric conditions.

The invention is illustrated by the accompanying drawings.

Of these drawings, Figure 1 is a side view of one shape of former, and Fig. 2 is a section of a metal reflector formed by dipping said former in a bath of molten metal or alloy. Figs. 3 and 4 are views, corresponding to Figs. 1 and 2, illustrating another shape of former and a reflector made by means thereof.

In both cases *a* is the head or main part of the former, which is provided with a smooth and highly polished surface, *b* are the stems by which the formers are held while they are dipped in a bath of molten metal or alloy, and *c* is a metal reflector formed by said dipping.

The manner in which the formers are used will be readily understood from an inspection of the drawings and the description of the method of carrying out the invention. It will be understood that the surface *b* of the formers must not only be clean but be absolutely free from any grease spots, and that if the shell obtained by once dipping a former is not of sufficient thickness the latter may be increased by dipping the shell, while adherent to the former, one or more times in the bath.

Having now described my invention, what I have invented and desire to secure by Letters Patent of the United States is as follows:—

1. A method of making metal reflectors or mirrors, consisting in the momentary immersion in molten metal of a former having that part of its surface intended to be immersed highly polished and formed of a shape the reverse of that of the reflecting surface of the reflector or mirror to be produced, and the separation of the solidified coating of metal from the immersed surface of the former after withdrawal of the latter from the molten metal.

2. A method of making metal reflectors or mirrors, consisting in the momentary immersion in molten metal or an alloy of low melting point of a former having that part of its surface intended to be immersed highly polished and formed of a shape the reverse of that of the reflecting surface of the reflector or mirror to be produced, and the separation of the solidified coating of metal from the immersed surface of the

former after withdrawal of the latter from the molten metal.

3. A method of making metal reflectors or mirrors consisting in the repeated momentary immersion in molten metal of a former having that part of its surface intended to be immersed highly polished and formed of a shape the reverse of that of the reflecting surface of the reflector or mirror to be produced and the separation of the solidified coating of metal from the repeatedly immersed former after its withdrawal on final immersion in the molten metal.

4. A method of making metal reflectors or mirrors consisting in the momentary immersion in molten metal after the scum has been removed from its surface to present a clean face of metal, of a former having that part of its surface to be immersed highly polished and formed of a shape the reverse of that of the reflecting surface of the reflector or mirror to be produced and the separation of the solidified coating of metal from the immersed surface of the former after its withdrawal from the molten metal.

5. A new article of manufacture being a solidified self-supporting film of metal, the whole of which is of the physical character of metal solidified directly from its molten state without mechanical treatment of any kind, the said solidified self-supporting film having one of its faces a mirror.

6. A new article of manufacture being a solidified self-supporting film of metal of low melting point, the whole of which is of the physical character of metal solidified directly from its molten state without mechanical treatment of any kind, the said solidified self-supporting film having one of its faces a mirror.

In testimony whereof I have signed my name to this specification.

THOMAS HANCOCK.